

April 3, 1934.

K. SCHUBERT

1,953,509

PROCESS FOR THE CARBONIZATION OF RAGS

Filed Dec. 31, 1931



Fig. 1



Fig. 2

INVENTOR

KARL SCHUBERT

By *A. M. Deller*

## UNITED STATES PATENT OFFICE

1,953,509

PROCESS FOR THE CARBONIZATION  
OF RAGS

Karl Schubert, Seon-Seetal, Switzerland, assignor to Max Gessner, Wiesbaden-Biebrich, Germany

Application December 31, 1931, Serial No. 584,139  
In Germany January 2, 1931

3 Claims. (Cl. 8—12)

Various processes are known for the carbonization of rags, that is, the isolation of their animal wool constituents by the destruction of the cotton and other vegetable or cellulosic constituents contained in the rags by means of acids and the like. According to the so-called wet carbonization method, the rags are impregnated with liquid acid, are thereupon freed from excess of acid by centrifuging or by steam treatment and are then carbonized. This process has not been found to be particularly satisfactory, chiefly because it requires comparatively much time, is expensive and does not always permit the desired carbonization effect to be attained in a uniform and certain manner. According to another known process, the rags are treated with hydrochloric acid gas. In such a process, however, there is the disadvantage of the danger in handling this gas and the difficulty that the rags must first be thoroughly and uniformly moistened, since hydrochloric acid gas alone as such does not act upon the rags.

In practice, therefore, the procedure has generally been first to dry the rags in a so-called carbonization drum and then to carbonize them by introducing acid vapours produced outside the treatment vessel, for example in a retort. However, even this process which, in itself, undoubtedly leads to satisfactory carbonization effects, is accompanied by considerable disadvantages and difficulties, chiefly consisting in the fact that the acid vapours produced with a considerable expenditure of heat and by means of particularly expensive apparatus at very high temperatures for example of about 800° C., have an extraordinarily corrosive action and thus comparatively very soon destroy the production and treatment apparatus, and are a source of danger to the attendants.

It has now been found that all the aforementioned difficulties and disadvantages may be eliminated and excellent carbonization effects may be attained with but slight expenditure of material and heat and in simple apparatus, which is practically not subjected to any wear, if the rags are first dried in known manner in a carbonizing drum and the acid, for example hydrochloric acid or sulphuric acid, is then introduced into the heated carbonizing drum in a liquid form and in a finely divided condition, for example by injecting it through nozzles. The temperatures of the treatment within the drum, when for example hydrochloric acid is used as the carbonizing acid, need not in general exceed 55 140° C. This process will be explained more

particularly hereinafter with reference to the accompanying drawing wherein

Figure 1 shows diagrammatically in plan by way of example an apparatus for carrying out the present process, and

Figure 2 shows the same in cross-section.

After the drum 1 has been made accessible by opening the two covers 2 and has been filled with rags, the covers 2 are again closed and the heating device, in this case a gas heating device 3, is set in operation, so as first of all to remove the natural moisture contained in the rags. At the same time, the heated air ascends in the heating chamber 4 and sweeps round the whole of the outer wall of the chamber 5 containing the drum 1. The interior of the drum and the rags contained therein are thereby also heated rapidly and the moisture is expelled from the rags. The excess of heating gases can escape through the pipe 6 and the evaporated moisture through the pipe 7. If heating is effected electrically or by means of steam, the pipe 6 may be dispensed with.

When the moisture has been expelled from the rags to a sufficient extent, liquid acid, for example hydrochloric acid, of the ordinary temperature is injected in a finely divided condition into the drum 1 through the nozzle 9 provided in one of the two stub axles 8 of the drum. The acid is supplied to the nozzle 9 through the conduit 10.

Figure 2 shows by way of example how the acid is led to the nozzle 9. The air compressor 12 is driven by the belt 11, the compressed air is led through the conduit 13 to the acid tank 14 and the acid is thereby forced through the supply conduit 10 to the nozzle 9. Preferably, the acid tank is protected against excessive pressure by means of a safety valve 15.

It is quite immaterial in itself what particular method is employed for injecting the acid, whether for example this is effected by means of compressed air or by means of a pump or the like. It is merely essential that the acid should reach the interior of the drum in a finely divided condition or in the form of a mist. The rags which are in the drum and which are continuously mingling with one another by the rotation of the drum, are thus able to come into uniform and intimate contact with the acid and the reaction between acid and rags can proceed rapidly and completely.

Before the introduction of the acid into the drum, the valve 16 of the outlet pipe 7 is closed, so that the chamber 5 is completely closed and

no acid vapours or dust can escape to the outside.

When carbonization is complete, the heating device 3 is shut off, whereupon the temperature falls comparatively quickly and any excess of acid there may be collects with the cellulose ash on the bottom of the chamber 5, whence it, like the carbonized material from the drum, can be removed easily and without inconveniencing the attendants.

*Example*

About 100 kilograms of rags are introduced into a carbonizing drum, perforated like a sieve, which is rotatably mounted within a heating chamber adapted to be suitably heated, for example by means of gas, steam or electricity, and is provided with an acid injecting device, for example a so-called atomizing nozzle, opening with in one of the stub axles of the drum. The drum and heating chamber are thereupon well closed, the drum is set in rotation, the air-release valve provided on the apparatus or on the heating chamber is opened, and the heating device is started. After the temperature in the drum has reached about 90 to 95° C., and the natural moisture has been driven out of the rags, this being accomplished in about  $\frac{3}{4}$  to 1 hour according to the size and type of the apparatus, the air-release valve is closed, and liquid hydrochloric acid of 22° Bé. and at the ordinary temperature is injected in a finely divided condition into the drum space through the acid injecting device in an amount of about 8 to 10% by weight of the rags, according to their nature. The temperature within the apparatus having been lowered somewhat by the introduction of the acid, is then raised by further heating to preferably about 90 to 140° C., and is maintained at this point until the carbonization process is completed, which is the case in  $\frac{3}{4}$  to 1½ hours, according to the nature of the rags and the size of the apparatus. The heating installation is then shut off, the air-release valve is opened, and any hydrochloric acid mist which may still be present is absorbed by filtering apparatus, con-

nected to the carbonization apparatus. After cooling, which in general does not take more than  $\frac{1}{4}$  hour, the rags which have been carbonized in an excellent manner with maximum protection to the apparatus material and small expenditure of heat and material, are then taken out.

I claim,

1. The process for the carbonization of rags which comprises heating said rags to dry them, treating said dried rags with liquid hydrochloric acid in a finely divided condition, continuing the heating, raising the temperature of said heating to a temperature not in excess of 140° C., continuing the treatment of said rags with liquid hydrochloric acid under said heat conditions until the rags are carbonized, and separating the carbonized rags from the acid. 85

2. The process for the carbonization of rags which comprises drying said rags to be carbonized, spraying said dry rags with liquid hydrochloric acid of about 22° Bé. strength in a finely divided condition, increasing the heat to a temperature not exceeding 140° C., continuing the spraying of said liquid hydrochloric acid under said heat conditions to effect the carbonization of the rags, cooling the carbonizing rags, and separating the carbonized rags from the acid. 90

3. The process for the carbonization of rags which comprises drying the rags at a temperature of about 90° C. to about 95° C. for a period of time extending up to about one hour, injecting liquid hydrochloric acid of about 22° Bé. strength as a fine spray on said dried rags, raising the heat to a temperature not exceeding 140° C., continuing the injection of said liquid hydrochloric acid under the aforesaid heat conditions for a period extending up to about one hour and one-half until the amount of injected hydrochloric acid approximates about 10% of the weight of the rags under treatment, cooling the carbonized rags for a period of time, said period being less than one hour, and separating the carbonized rags from the liquid hydrochloric acid. 105

KARL SCHUBERT. 110

120

50

125

55

130

60

135

65

140

70

145

75

150